

No. 874,380.

PATENTED DEC. 24, 1907.

A. J. BALDWIN.  
METHOD OF MAKING WIRE GLASS.

APPLICATION FILED AUG. 2, 1906.

2 SHEETS—SHEET 1.



Witnesses:  
Raphael Letter  
A. Dunham

A. J. Baldwin, Inventor,  
By his Attorneys  
Kerr, Page & Cooper.

No. 874,380.

PATENTED DEC. 24, 1907.

A. J. BALDWIN.  
METHOD OF MAKING WIRE GLASS.  
APPLICATION FILED AUG. 2, 1906.

2 SHEETS—SHEET 2.



Witnesses  
Raphael Ketter  
S. S. Dunham.

Inventor  
A. J. Baldwin  
By his Attorneys  
Kerr, Pass & Cooper

# UNITED STATES PATENT OFFICE.

ARTHUR J. BALDWIN, OF EAST ORANGE, NEW JERSEY.

## METHOD OF MAKING WIRE-GLASS.

No. 874,380.

Specification of Letters Patent.

Patented Dec. 24, 1907.

Application filed August 2, 1906. Serial No. 328,881.

*To all whom it may concern:*

Be it known that I, ARTHUR J. BALDWIN, a citizen of the United States, residing at East Orange, in the county of Essex and State of New Jersey, have invented a certain new and useful Method of Making Wire-Glass, of which the following is a specification.

My invention relates to the manufacture of sheet glass having embedded in it a strengthening structure, such, for example, as a meshed wire fabric, and known generally as "wire glass".

The object of my invention is to provide a rapid and efficient process which shall produce strong, homogeneous sheets, employing for the purpose apparatus of the simplest character.

The invention will be more readily understood when explained in connection with the annexed drawings. Therein,

Figure 1 illustrates, in diagrammatic longitudinal section, a convenient, simple and effective apparatus for practicing my method. Fig. 2 shows a preliminary stage in making a sheet of wire glass by my method, with the apparatus illustrated in Fig. 1. Fig. 3 is a diagrammatic longitudinal section of a modification of the apparatus of Fig. 1.

The apparatus shown in Fig. 1 consists of a longitudinally moving rolling-table, 1, and a forming-roll 2, spaced above the table a distance equal to the desired thickness of the finished sheet of glass. Back of the first is another roll, 3, near enough to the first roll to form a sort of hopper between them, so that a batch of plastic glass deposited upon the rolls, between them, will spread across the same and descend between the rolls evenly across the table, as will be readily understood. The roll 3 is so spaced from the table that the distance between its periphery and the table is substantially the distance from the table to the position which

it is desired the wire fabric should occupy in the sheet of glass. The table 1 and roll 2 are driven in the direction of the arrows by any convenient means, not shown, such that the lineal speed of the former and the peripheral speed of the latter are the same. The roll 3 is rotated preferably at the same speed. Under the last mentioned roll passes a strip 4 of the fabric which is to be embedded in the sheet of glass, the said fabric being drawn from any suitable supply, as the roll

5 thereof, and requiring a certain tension to draw it off said roll 5.

The wire fabric is passed under the roll 3 and its end may be allowed to fall upon the table near the roll 2. A mass of plastic glass 6 is then deposited between the rolls 2 and 3 and is from them deposited upon the fabric, the glass being sufficiently molten to pass more or less freely by its own weight through the meshes of the fabric. The condition at this stage is shown in Fig. 2. The end of the strip being held by the weight of the glass on the same, the tension of the fabric lifts it gradually and holds it above the table and against the roll 3 and allows the glass to pass through the meshes of the fabric instead of bearing it down upon the table. The movement of the table 1 and the roll 2 draws out the lower portions of the mass of glass into a sheet 7, as will be readily understood, carrying the fabric with it, while the fabric assumes in the sheet a position like that shown in Fig. 1, at about the same distance above the table as the space between the table and the roll 3, this position being maintained as the roll and table continue to draw out the portions of the mass above and below the fabric. The reason for the fabric assuming such position seems to be due to a seeking of the "path of least resistance", since the upper and lower surfaces of the sheet being slightly chilled by the roll and table, the central portion of the sheet is the softer and hence offers least resistance to the movement of the fabric in its tendency to assume a tangential position to the roll 3 from the point at which the tension is exerted, namely, between the roll 2 and the table. But be that as it may, it is a fact that the fabric seeks the center of the space between the roll 2 and table 1, and assumes a position within the sheet there formed. The end of the fabric may, however, be positively held at the desired distance above the table by means of a clamp, not shown, or other suitable means.

As the sheet is drawn out, and with it the fabric, the glass keeps falling through the fabric at the rear of the mass, keeping the quantity below the fabric substantially the same. As the mass of glass 6 becomes smaller and smaller, it may, if desired, be replenished from time to time. In this way the process may be continuous and the length of the sheet would be limited only by the length of the table; but by using a succession

of tables, one behind the other, a sheet of any desired length can be produced, as will be readily understood. When the sheet is finished the table bearing the same may be 5 transferred to the annealing oven for the usual annealing.

In the apparatus shown in Fig. 3 the function of the plane rolling-table 1 is performed by a rolling table of cylindrical form, as the 10 roll 9, the process, however, being essentially the same. The sheet formed between the rolls 2 and 9 leaves the latter at or somewhat below the horizontal diameter of the same and is received by any suitable means, as an 15 annealing table 10.

Wire glass made by this process is equal in every respect to the product of any other process or apparatus with which I am familiar. At the same time the process is rapid 20 and, as is evident from the foregoing description, can be practiced with apparatus of a very simple character.

What I claim is:

1. The herein described method of making 25 wire glass, which consists in depositing between oppositely rotating rolls and upon a longitudinally movable wire fabric passing under said rolls a mass of glass sufficiently

plastic to pass by its own weight through the spaces or meshes of the fabric, whereby the 30 latter is embedded in the glass, and progressively drawing out from the mass of glass portions thereof on both sides of the fabric, simultaneously advancing the fabric and causing a continual passing of glass through 35 the fabric at the rear of the mass, as set forth.

2. The herein described continuous process of making wire glass, which consists in depositing between oppositely rotating rolls 40 and upon a longitudinally movable fabric passing under said rolls a mass of glass sufficiently plastic to pass by its own weight through the spaces or meshes of the fabric, whereby the latter is embedded in the glass; 45 and progressively drawing out from the mass of glass portions thereof on both sides of the fabric, simultaneously advancing the fabric and causing a continual passing of glass through the fabric at the rear of the mass; 50 and replenishing the mass of glass from time to time as required; as set forth.

ARTHUR J. BALDWIN.

Witnesses:

S. S. DUNHAM,  
ARTHUR E. MAHAN.